

## UNITED STATES PATENT OFFICE

FREDERICK E. KERN, OF ST. LOUIS, MISSOURI

## PROCESS OF MANUFACTURING FUELS

No Drawing.

Application filed June 18, 1930. Serial No. 462,132.

This invention relates to a smokeless fuel, and with regard to certain more specific features, to a smokeless fuel made from vegetable materials, for example, wood.

5 Among the several objects of the invention may be noted the provision of a smokeless fuel of the class described which is firm and hard and wear-resisting; a fuel of the class described which, when burned, forms a porous, heat-retaining and heat-radiating sponge which, however, is reduced to a powdered ash with minimum trouble; a fuel of the class described which is easily ignitable, and forms a suitable material for starting fires with less 10 easily ignitable fuels; the provision of a process for manufacturing a fuel of the class described which provides for the recovery of valuable volatile products; a process of the class described which permits of the formation of the fuel in regular shapes or briquettes; and a process of the class described which is easily and economically carried through with a minimum use of expensive 15 treating materials. Other objects will be in part obvious and in part pointed out herein-after.

20 The invention accordingly comprises the elements and combinations of elements, steps and sequence of steps and features of synthesis which will be exemplified in the description hereinafter and the scope of the application of which will be indicated in the following claims.

25 Fuel materials made from comminuted vegetable materials in which binders of molasses, pitch, tar, asphalt, water glass, and the like are used, are known to the art. Such fuels, employing carbonaceous materials as binders, are objectionable in that they burn with a smoky, sooty flame. Fuels employing water glass binders are objectionable in that they are difficult to ignite, on account of the well-known fireproofing qualities of said water glass. The present fuel overcomes said 30 difficulties by presenting a binder material of non-combustible, inorganic, plasticizable material which does not retard ignition or combustion.

35 In carrying out the invention, comminuted vegetable materials, such as wood fines or

sawdust, are mixed with a binder material such as comminuted earthy materials, for example, carbonaceous shales, clays, and the like, having a high alkaline-earth metal content. The mixture is then treated with a 55 suitable plasticizing agent, which, according to the characteristics of the binder material, may be water, acids, chloride solutions, or alkaline solutions. With suitable homogenizing, as in a pug mill or wet pan, the comminuted binder material is rendered plastic with the plasticizing agent. The plastic binder material encloses the wood fines and renders the mass as a whole plastic and moldable. 60

45 As plasticizing agents, I have found water to be generally successful, and especially successful in combination with binder materials having high aluminum hydroxide and colloidal silica contents, such as carbonaceous 70 shales and clays. Acids and chloride solutions are of especial value in combination with binders having a high alkaline-earth metal content; alkalies are similarly of especial 75 value with binders having high silica contents.

50 The plastic mass of wood fines and binder material is next formed into shapes or briquettes, for example, by a ceramic extrusion machine. The shapes or briquettes are then 80 preferably dried. The dried briquettes are charged into a distillation retort, wherein they are destructively distilled at temperatures up to the order of 500° C. Attendant upon the distillation is an evolution of volatile products, which include both condensable, and, under the ordinary use of the term, non-condensable vapors. These volatile products are condensed where practicable, and the non-condensable products are used for heating the 85 retort and the like. The condensate includes such valuable compounds as methanol, acetone, acetic acid, wood tar, and hydrocarbons. 90

55 Subsequent to the distillation, which is terminated upon the substantial cessation of 95 the evolution of vapors, the briquettes are cooled and the cooled briquettes comprise the fuel product. This fuel product is in the nature of a char, interspersed with and hardened by the inorganic binder material, 100

50

- which is now present as a hardened structural or skeletal binder. The fuel is easily ignitable, due to the absence of combustion-retarding materials. Upon ignition the char material burns, and when entirely burned, leaves a highly porous sponge of inorganic material which is both heat-retaining and heat-radiating. The inorganic sponge holds its shape until broken down, as with a poker, into a fine ash powder. It is to be understood that this inorganic sponge is not hard in the nature of a clinker, requiring considerable breaking force, but, on the contrary, is easily broken down with a minimum of force.
- 15 It is to be understood herein that vegetable materials generally, such as corn cobs, straw, sugar cane trash, tannery waste, and like cellular materials may be used in place of the wood fines described.
- 20 In view of the foregoing, it will be seen that the several objects of the invention are achieved and other advantageous results attained.
- 25 As many changes could be made in carrying out the above objects without departing from the scope of the invention, it is intended that all matter contained in the above description shall be interpreted as illustrative and not in a limiting sense.
- 30 I claim:
1. The process of manufacturing fuels, which comprises comminuting a vegetable material, mixing therewith a binder material such as carbonaceous shales, clays, and the like, particularly those having a high aluminum hydroxide or colloidal silica content, comprising a comminuted earthy material, plasticizing the mixture with water, forming the plastic mixture into shapes, and subjecting said shapes to a destructive distillation.
  2. The process of manufacturing fuels, which comprises comminuting a vegetable material, mixing therewith a binder material comprising a comminuted earthy material such as carbonaceous shales, clays, and the like, particularly those having a high alkaline-earth metal content, plasticizing the mixture with acids, forming the plastic mixture into shapes, and subjecting said shapes to a destructive distillation.
  3. The process of manufacturing fuels, which comprises comminuting a vegetable material, mixing therewith a binder material comprising a comminuted earthy material such as carbonaceous shales, clays, and the like, particularly those having a high silica content, plasticizing the mixture with chloride solutions, forming the plastic mixture into shapes, and subjecting said shapes to a destructive distillation.
  4. The process of manufacturing fuels, which comprises comminuting wood, mixing therewith comminuted carbonaceous shale, plasticizing the shale with water whereby the

mixture becomes plastic, forming the plastic mixture into briquettes, drying said briquettes, and subjecting said dried briquettes to a destructive distillation at temperatures up to the order of 500° C., whereby condensable and non-condensable vapors are produced, condensing said condensable vapors, and cooling said distilled briquettes.

In testimony whereof, I have signed my name to this specification this 13th day of June, 1930.

FREDERICK E. KERN.

80

85

90

95

100

105

110

115

120

125

130